

June 7, 1927.

1,631,550

P. ROBERG

ELECTRICAL CONNECTION

Filed Aug. 26, 1921



Inventor:

Philip Roberg,  
J. Byman, Townsend & Bickersteth,  
Attorneys.

## UNITED STATES PATENT OFFICE.

PHILIP ROBERG, OF ELMHURST, NEW YORK, ASSIGNOR, BY MESNE ASSIGNMENTS, TO NATIONAL CARBON COMPANY, INC., OF NEW YORK, N. Y., A CORPORATION OF NEW YORK.

## ELECTRICAL CONNECTION.

Application filed August 26, 1921. Serial No. 495,499.

This invention relates to the attachment of electrical conductors to current receiving members and has particular reference to improvements in means and compositions for securing flexible cable connections to the commutator brushes of dynamo-electric machines.

Brushes of this type are as a rule subjected to substantially continuous vibration and it has proved difficult to connect a wire or cable to them so that it will not work loose during service, resulting in an increase of resistance and undue heating. Securing the cable by means of bolts, rivets, or the like, materially complicates the manufacture of the brush. A simpler method which has been proposed is to embed the end of the flexible connector in solder or other easily fusible alloy. Such connections are not reliable, however, for the reason that brushes are likely to be heated by the current to a temperature above the melting point of the alloy.

The patent to H. B. Eynon, No. 1,188,635, dated June 27, 1916, describes a carbon brush connection involving the use of copper amalgam as a cementing means for attaching the cable to the brush. The process outlined in this patent enables a relatively satisfactory connection to be made in a very simple manner. I have discovered, however, that by a modification of the composition of the amalgam and certain other procedures relating to its use, I secure a connection of substantially diminished resistance during service and greater strength.

The present invention consists broadly in the use of carbon, preferably in the form of graphite, with copper amalgam which may be of the type described in the above-mentioned patent to Eynon, or with any metallic packing material suitable for securing a cable to a brush, for example, compacted copper powder.

The invention will be described in detail in connection with the accompanying drawings, in which

Fig. 1 is a vertical section through a brush carrying a cable attached according to a preferred form of my invention, and

Figs. 2 and 3 are vertical sections through brushes showing modified forms of holding means.

Referring to the drawings, the flexible

conductor 1 is shown as formed as usual of braided copper wire, but any desired type of conductor may be used. The brush 2 may consist of any suitable composition of comminuted carbon held together by a binder and may contain graphite, copper or other electrically conductive materials.

The invention is not limited to any particular form of brush cavity designed to receive the end of the cable. The connection may advantageously be made by drilling a straight cylindrical hole of suitable diameter through the top of the brush, and of a depth depending on the size of the brush. The end of cable 1 is inserted centrally in the drilled hole and the connection is completed by filling the cavity about the cable with a carbon-containing compactible metallic substance, which serves as a composite electrical and mechanical bond holding the cable securely in the brush. Electroplating of the hole is not essential to the successful use of my invention, but it may be employed.

Various amalgams, or metals in the form of compactible powders or filaments, can be used, but a copper or copper bronze amalgam is preferred. The amount of graphite mixed with the metal or amalgam may be adjusted so as to obtain a connection of the desired type. For example, in cases where an especially high "pull out" resistance is not demanded, the graphite content may advantageously be around 10%. This proportion of graphite in the metallic packing insures a continuous low resistance connection throughout the service of the brush, and the strength of the connection is substantially equal to those made with metal alone. Tamping of the bonding mixture into the brush opening is considerably facilitated by the presence of such relatively large amounts of graphite. The strength of the bond is somewhat greater, however, when lower percentages of graphite are used. I have found that the admixture of about 2½% of graphite in general gives a maximum with respect to both strength and conductivity during service.

The stated percentages are, of course, illustrative only, and may be varied in accordance with the particular character of connection desired.

A typical cementing amalgam may be

prepared by mixing 100 parts by weight of copper or copper bronze powder and 25 parts of mercury, stirring with dilute sulfuric acid to a pasty consistency and rubbing the mixture thoroughly until amalgamation is complete, after which the acid is removed by washing. At this stage the amalgam is porous and plastic, and 3 parts by weight of graphite are added with thorough mixing. When tamped into the brush cavity, this forms a coherent mass or plug of high electrical conductivity between the cable and the carbon or its electroplated surface.

15 The amalgam described expands to an extent sufficient to bind the cable firmly in the brush cavity. In addition, a superficial amalgamation of the strands of the conductor and the copper plating occurs, tending also to hold the parts together by the merging of the amalgam filling into the metals adjacent it.

Instead of incorporating the graphite in the amalgam, a coating 5 of graphite may be applied to the cavities, which need not be electro-plated, as shown in Fig. 2. This coating may be advantageously applied by swabbing the walls of the cavities with graphite. The thickness of the coating may 30 be varied, but a relatively thin layer is preferable and substantially prevents the formation of a high resistance contact, which is likely to occur when copper amalgam containing no graphite is applied directly to the surface of the brush cavity. When the graphite coating is applied, the amalgam need not contain carbon, but the graphite-copper amalgam above described, or others of its type, may of course be used if desired.

40 In the form of my invention illustrated in Fig. 3, a layer 6 of graphite is tamped about the lower end of the flexible conductor. Any suitable conductive bonding material 7, which may advantageously be a metal or amalgam packing, is placed above layer 6. The packing may contain graphite as described above, but in general this will be omitted as the primary purpose of the metal or amalgam is to make a bond of adequate strength between the brush and the conductor. The use of the graphite layer ensures a continuous low resistance contact during service.

55 My invention consists broadly in the formation of a composite electrical and mechanical bond between carbon brushes and conductors by the joint use of graphite and a conductive bonding material, especially a metallic packing. Various specific embodiments of this general idea, other than those herein described, are within the scope of the appended claims.

I claim:

1. The combination of an electric brush

having a cavity therein, a conductor extending into said cavity and a composite electrical and mechanical bond between the brush and the conductor, said bond including a metal and graphite.

2. The combination of an electric brush having a cavity therein, a conductor extending into said cavity, a metal-containing plug for securing the conductor in the cavity, and graphite associated with said plug to reduce the electrical resistance between the conductor and the brush during service.

3. The combination of a carbon brush having a cavity therein, a carbon-containing metallic plug in said cavity and a conductor secured in good electrical connection with the brush by the metallic plug.

4. The combination of a carbon brush having a cavity therein, an electro-plated lining for said cavity, a conductor projecting into said cavity and a carbon-containing amalgam plug establishing good electrical and mechanical connection between said conductor and carbon.

5. The combination with an electric brush having a cavity therein, of a conductor having an end inserted in said cavity, said end being embedded in a layer of graphite and a layer of a metallic bonding substance.

6. The combination with an electric brush having a cavity therein, of a conductor inserted in said cavity, a layer of graphite establishing electrical connection between the lower portion of the conductor and the brush, and a conductive bonding material above said graphite layer.

7. The invention according to claim 6, in which the bonding material is a compactible amalgam.

8. In combination, a brush, a conductor therefor, and a plug of metal-graphite composition for retaining the conductor in an opening in the brush.

9. In combination, an electric brush having an opening, a conductor having a portion extending into said opening, and an amalgam-graphite bond in said opening for retaining said portion of said conductor in said opening.

10. The invention according to claim 9, wherein the graphite content of said bond is relatively low.

11. The invention according to claim 9, wherein the graphite content of said bond is not greater than about 10% by weight, the remainder being amalgam.

12. The invention according to claim 9, wherein the graphite content of said bond is about 2.5% by weight, the remainder being an amalgam comprising a mixture of copper powder and mercury.

In testimony whereof, I affix my signature.

PHILIP ROBERG,